

Oct. 14, 1947.

**C. WESSEL**

2,429,145

## MOLD FOR CASTING METALS

Filed Dec. 26, 1942

5 Sheets-Sheet 1



Inventor.

Carl Wessel  
By Mc Caleb, Heriot & Dickinson  
At 185

Oct. 14, 1947.

C. WESSEL

2,429,145

### MOLD FOR CASTING METALS

Filed Dec. 26, 1942

5 Sheets-Sheet 2



Oct. 14, 1947.

C. WESSEL

2,429,145

MOLD FOR CASTING METALS

Filed Dec. 26, 1942

5 Sheets-Sheet 3



Inventor  
Carl Wessel  
By Carl Wessel  
770 Calle, San Joaquin  
Signature

Oct. 14, 1947.

**C. WESSEL**

**2,429,145**

## MOLD FOR CASTING METALS

Filed Dec. 26, 1942

5 Sheets-Sheet 4

Fig. 5.



Inventor.  
Carl Wessel  
By  
McCaleb, Wendt & Dickinson  
St. Louis.

Oct. 14, 1947.

C. WESSEL

2,429,145

MOLD FOR CASTING METALS

Filed Dec. 26, 1942

5 Sheets-Sheet 5

Fig. 8.



Fig. 9.



Fig. 10.



Fig. 11.



Inventor:  
Carl Wessel  
By McColl, Knudt & Dickenson  
Attn: J. S. A. S.

## UNITED STATES PATENT OFFICE

2,429,145

## MOLD FOR CASTING METALS

Carl Wessel, Chicago, Ill., assignor to himself and  
Lew W. Cleminson, Chicago, Ill., as trustees

Application December 26, 1942, Serial No. 470,167

4 Claims. (Cl. 22—145)

1

The present invention relates to an improved method for making thin metal sheets or thin plates, and is particularly concerned with the provision of a method by means of which such metal sheets or plates may be formed of homogeneous large-grained structure without segregated impurities and with a minimum amount of impurities of any kind.

The present application is a continuation-in-part of my prior application which resulted in U. S. Patent No. 2,333,286, issued November 2, 1943, and application Serial No. 370,344, filed December 16, 1940, for Method and apparatus for making drawn metal tubes and metal castings, which resulted in U. S. Patent No. 2,309,608, issued January 26, 1943.

One of the objects of the invention is the provision of an improved method of casting and treating metals such as clean scrap or any other metal in ingot form by means of which plates or sheets of metal may be made which have a homogeneous large-grained structure and which are substantially free from segregations or impurities.

Another object of the invention is the provision of an improved method of the class described by means which cast metal plates or rolled sheets may be made which have a substantial increase of tensile, compression and shearing strength and which have the characteristic of a better degree of workability than the metals made according to the methods of the prior art.

Another object of the invention is the provision of an improved method of making drawn tubular members by means of which the imperfections and defects of the tubular members made according to the prior art may be eliminated.

Another object of the invention is the provision of an improved and simpler method of making drawn tubular members by means of which the step of preheating may be eliminated and by means of which such tubular members may be drawn with less difficulty and less imperfections than those which are produced according to the methods of the prior art.

Another object of the invention is the provision of an improved method of casting by means of which the defects of the prior art methods, such as blow-holes, inclusions, segregations, faults, cracks, and other defects, are practically eliminated.

Another object of the invention is the provision of an improved casting method which is adaptable to use in small or large plants and which is adapted to produce metallic members having the characteristics of high degree of uniformity of

2

crystalline structure and a uniform smooth outer surface adapted to be polished without necessity for smoothing the surface after casting and before the polishing.

5 Another object of the invention is the provision of an improved method of casting by means of which tubular structures may be made having a high degree of uniformity of crystalline structure and by means of which they may be constructed at a minimum cost.

10 Another object of the invention is the provision of an improved method of producing a superior cast metal product or a sheet metal product which is simple and which involves a minimum number of operations and the apparatus of which may be made very simple so that a minimum amount of capital and labor is required in the production of the articles made by the process.

15 Other objects and advantages of the invention will be apparent from the following description and the accompanying drawings, in which similar characters of reference indicate similar parts throughout the several views.

*The drawings*

25 Referring to the five sheets of drawings:

Fig. 1 is a fragmentary, front elevational view of a casting apparatus embodying the invention;

Fig. 2 is a similar side elevational view of the 30 casting apparatus;

Fig. 3 is a vertical sectional view taken on the plane of the line 3—3 of Fig. 1, looking in the direction of the arrows, showing the details of structure and interior shape of the mold and ladle;

35 Fig. 4 is a horizontal sectional view taken on the plane of the line 4—4 of Fig. 3, looking in the direction of the arrows;

Fig. 5 is a view similar to Fig. 3, with the parts of the apparatus in the position which they assume during the casting of a thin metal plate;

Fig. 6 is a fragmentary top plan view of the ladle and its cover, with the mold removed;

Fig. 7 is a diagrammatic sectional view taken 45 on the plane of the line 7—7, looking in the direction of the arrows, of Fig. 6, with the mold shown in dotted lines, showing its position relative to the ladle;

Fig. 8 is a diagrammatic vertical sectional view, 50 taken on a plane passing through the axis of the ladle at right angles to the plane of the casting, showing the ladle and mold in vertical position, before the casting operation;

Fig. 9 is a similar view, with the ladle and 55 mold tilted to such a point that the flame of the

burner is cut off from the mouth of the mold, as takes place in the beginning of the casting operation;

Fig. 10 is a similar view, with the mold and ladle tilted still farther until the free surface of the metal has begun to well up into the mold;

Fig. 11 is a similar view, showing the ladle and mold in a further tilted position, with the free surface of the metal more than half way up into the mold;

Fig. 12 is a similar view, showing the ladle and mold tilted still further until the free surface has welled up to the very top of the mold and the mold is full;

Fig. 13 is a similar view, showing the final position to which the ladle and mold are usually tilted, with the mold substantially horizontal and all parts of the mold located substantially below the main body of the metal in the ladle.

In order to illustrate the preferred means for carrying out the method, one form of apparatus or casting machine capable of practicing the method is now described in detail.

Referring to Figures 1 and 2, the casting apparatus which has been selected to illustrate the invention, preferably includes a movably supported ladle indicated in its entirety by the numeral 10, and a mold 11 directly connected to the ladle 10 and adapted to be moved with it. The ladle 10 is preferably movably mounted on a pair of bearing frame members 12, 13 and is preferably so balanced with respect to the assembly of the mold 11 and ladle 10, that it will be normally held in upright position as shown in Figures 1 and 2, even when the supply of molten metal in the ladle has been exhausted.

The bearing brackets 12 and 13 may be identical in shape and construction and therefore only one of them need be described in detail. These brackets are preferably of sufficient length to permit a maximum degree of pivotal movement of the ladle and mold and may, in some embodiments of the invention, permit full rotation of the mold and ladle throughout 360°. This may be accomplished by providing a pit in the floor 14 between the frame members 12 and 13 and extending forwardly and rearwardly of them, or the frame members 12 and 13 may be supported in elevated position upon blocks 15 as shown in Figure 5.

Each frame member preferably has a pair of upwardly extending columns 16, 17, integrally supported by a bottom frame member 18 which has a pair of attaching flanges 19, 20, provided with apertures for receiving the bolts or lag screws 21. The frame members 16-18 may be substantially T-shaped in cross-section and at the upper end of the bearing brackets 12 and 13 they are formed with the rectangular opening 22 defined by the frame portions 23-26.

The frame portions 23-26 are preferably provided with threaded apertures for receiving the screw bolts 27-32. Each screw bolt 27 has its inner end engaged in a socket 33 in one of the bearing blocks 34, 35, and the screws are held in fixed position by lock nuts 36.

The bearing blocks 34, 35 comprise a pair of metal members which, when assembled as shown in Figure 2, have plane rectangular sides and are formed with a bearing aperture 37. Since the bearing blocks 34, 35 are adjustably supported by the screw bolts 27-32, they may be brought into alignment even after the frame members 12 and 13 have been secured in place, provided the frame members are also substantially in alignment.

The ladle 10 may comprise a substantially cylindrical metal shell, such as the shell 38, having the cylindrical side walls 39 and flat bottom 40. This metal shell may be lined with a layer of suitable insulating material, such as asbestos 41, covering the inner surface of its side walls 39 and its bottom 40.

The asbestos lining 41 supports a second rigid lining 42 of a refractory material, such as a ceramic product adapted to withstand the melting temperatures to which the metal is to be subjected. This ceramic lining 42 is provided with an inner chamber 43 which may be substantially cylindrical in shape except that the lower corners are rounded at 44, 45 and the left-hand wall 46 (Figure 3) may be tapered or may be made substantially frusto-conical at its lower portion leading to a substantially frusto-conical cover opening 47 at the top.

The opening 47 for the cover plug 48 diverges from the cylindrical shape at the left-side where it may be provided with a flat wall surface at 49 for cooperating with the cover plug 48 to form the walls of a rectangular aperture 50 in the top of the ladle 10.

The cover plug 48 may comprise a frusto-conical member of refractory material, such as the same ceramic 42 which is formed to fit in the frusto-conical opening 47 over the major portion of its outer frusto-conical surface 51. At the right-hand side, the cover plug 48 is formed with a groove 52 which is half-circular at the upper end and which increases in size frusto-conically toward the bottom of the plug. When the plug 48 is assembled with the ladle 10, the aperture 52 at the right-hand side is adapted to provide an upwardly tapered conduit for receiving the burner flame 53 which may be directed downwardly into the ladle from the gas burner 54 to apply heat to the surface of the metal and to be reflected upwardly into the mold 11.

At its left side (Figure 4) the cover plug 48 is formed with a groove 50 which is rectangular in cross-section and which at its upper end forms a discharge opening 55 of the same size as the filling opening of the mold 11 to which it is directly connected. The rectangular groove 50 in the cover plug 48 may increase in depth and width toward the bottom of the plug 48 (Figure 3) so as to provide a tapered conduit 56 in this side of the ladle leading from the chamber 43 to a discharge aperture 55 which is coincident with the filling aperture of the mold.

The shell 38 of the ladle 10 is preferably supported in a basket-like metal frame which may consist of a metal hoop 51, and a plurality of longitudinally extending metal straps 58-61 which have inwardly turned ends 62 at their lower end for attachment to the bottom of the shell 38. A transversely extending bar 63 is carried by the bottom of the shell 38 and is adapted to be engaged by a latching lever 64 which is pivotally mounted by means of a bolt 65 on one of the legs 17 of the frame member 13.

The latching bar 64 has a slot 66 which engages the bar 63 when the ladle is in vertical position as shown in Figure 2, to retain it in this position against any possibility of moving or tipping. A tension coil spring 67 has one end secured to the frame member 13 at the bolt 30 and the other end pivotally secured to the latching lever 64 by means of a block 68 secured to the end of the spring and pivotally mounted by means of the pivot pin 69. The latching lever is thus urged

into latching position shown in full lines in Figure 2 but may be moved out of engagement with its keeper 63 by pressing downward on the latching lever 64 with the foot.

The hoop 57 is secured to the vertical frame members 58-61 at their intersection by suitable bolts or by welding, and the vertical frame members 58-61 may be turned outwardly at their upper ends and secured by means of bolts to a cover plate 70 which may project beyond the outer wall of the shell 38 sufficiently to engage the laterally turned ends 71 of the frame members 58-61.

The cover plate 70 is provided with a rectangular aperture 72 located to register with the discharge aperture 55 in the ladle 10 and plug 48 and the conduit extending through the cover plate 70 is made continuous and smooth from the conduit 56 into the filling opening of the mold 11, the aperture 72 being of the same size as the filling opening of the mold 11.

The cover plate 70 holds the plug 48 firmly in place and it is also provided with an aperture 73 (Figure 5) for passing the gas burner nozzle 54. The bolts 74 which secure the frame members 58-61 to the cover plate 70 may also be used to secure to the top of the cover plate a plurality of metal bars 75-79. These metal bars may be of rectangular section and they are a part of the structure utilized with other bars for securing the mold directly to the top of the ladle.

For example, the metal bar 75 may be secured to the cover plate 70 by a plurality of bolts passing through the bar and threaded into the cover plate and the bar 75 is preferably located with its inner face 80 substantially parallel to both of the edges of the discharge aperture 72 as it is intended to hold one-half of the mold 11 in proper position in registry with the aperture 72 at its lower end.

The mold 11 comprises a pair of parts 81, 82 and the lower and left corner 83 of the mold half 81 engages the face 80 of the bar 75. The bars 76 and 77 carried by the cover plate 70 are preferably elongated and extend forwardly from the ladle 10 over a length which is sufficient to support the half mold member 81 when it is in the position of Figure 2. For this purpose, the bar members 76 and 77 may be braced by having an upwardly extending frame member 84 at the end of each bar member 76, 77, the upper end of which is secured to another horizontally extending bar 85 by means of screw bolts 86. The bar members 76, 77 may be secured together at regularly spaced points by transversely extending bars 87, 88, 89 and the inner ends of the bars 85 may be secured to the fixed mold member 82 by a rivet or bolt 83.

The bars 76, 77 and the bars 85 are spaced from each other laterally sufficiently so that the mold member 81 may lie between them and the vertical frame members 84 project above the bars 85 to provide a stop surface 90 for engagement with the laterally projecting pipe 91 carried by mold member 81. Thus, the mold member 81 is prevented from sliding endwise toward the left off the supporting frame which comprises the bars 76, 77, 85, 84 and others.

The horizontal supporting frame for the mold member 81 may be indicated in its entirety by the numeral 92. The mold member 81 is preferably fixedly supported on the ladle 10 by means of a vertically extending frame on each side. This frame may consist of the vertically extending frame members 93-96 (Figure 6) which are

secured to the horizontally extending bars 97, 98 on the cover plate 70.

The bars 93, 94 are secured together at regularly spaced points and the bars 95, 96 are secured together at regularly spaced points by means of screw bolts and horizontal frame members 99-101. The frames at each side are secured together by the transversely extending frame member 102.

The uppermost transverse frame members 99 (Fig. 3) are joined by a frame member 103 which may have a beveled surface 104 on the side which engages the fixed mold member 82. The fixed mold member is preferably substantially rectangular in elevation and comprises a metal member provided with a plane, smooth and polished surface 105 forming one of the sides of the mold cavity 106.

The two mold members 81 and 82 are made of metal having a higher melting point than the metal which is to be cast into plates. For example, when casting aluminum and certain other alloys, cast steel molds may be used. The mold member 82 is preferably provided with a rearwardly extending reinforcing border flange 107 extending on all the four edges of the body plate 108 and it is also preferably provided with a plurality of transversely extending reinforcing ribs 109. Vertically extending reinforcing ribs may also be employed for the purpose of preventing the warping of the mold, and the lower edge of the fixed mold 82 is preferably beveled as at 110 so that it will fit against the cover plate 70 when the mold is disposed at an angle as shown.

The face 105 of this mold 82 registers with the opening 72 in the cover plate 70 which in turn registers with the discharge opening 55 from the chamber 43 of the ladle. The width of the mold members 81, 82 is such that the mold cavity 106 is as wide as the discharge openings 72 and 55 are long. The thickness of the mold cavity 106 is the same from top to bottom and is of such thickness that the lower open end of the mold has the walls of its cavity in registry with the edges of the opening 72 in the cover plate 70.

The fixed mold 82 rests against the frame member 103 at the top and against the cover plate 70 at the bottom and is preferably secured in place by a plurality of screw bolts 111 extending through the frame members 99 and threaded into the flange 107 of the mold 82. Another pair of screw bolts 112 (Fig. 7) may pass through the lateral frame members 77 and may be threaded into the flange 107 (Fig. 5) of the mold 82 adjacent its lower end.

The movable mold member 81 preferably has a body portion which is similar in construction, being provided with a main body plate 113, a border flange 114 on all sides, and reinforcing flanges 115. This movable mold member, however, is preferably provided with a mold wall 116 which extends across the top of the mold member 81 and down both sides of the mold member 81, but is open at the bottom, thereby defining a mold filling opening 117. This mold member has its lower border flange 114 provided with an oppositely beveled surface 118 so that it may fit against the cover plate 70. The width of this surface 118 is such that when the toe 83 of the mold 81 engages the bar 75, the filling opening 117 is in registry with the opening 72 in the cover plate 70. Thus, the mold 11 is adapted to have a filling opening which is of substantially the same size as the discharge opening in the ladle,

the reasons for which will be described herein-after.

The movable mold 81 may be provided with a handle 91 which is of sufficient length to project laterally from both sides of the mold 81. It 5 may comprise a metal pipe which is secured to the vertically extending reinforcing flanges 114 (Fig. 1) by a plurality of screw bolts 120 which pass through apertures of the pipe and are threaded into the flanges 114. The handle 91 also 10 serves the purpose of providing a support for the mold 81 when it is moved into the dotted line position of Fig. 2, resting on the frame members 85 by means of handle 91.

The fixed mold 82 is preferably provided with means for holding the movable mold 81 in tight engagement with it as follows: At the upper end of the fixed mold 82, there is secured to its rear side on each of the reinforcing ribs 114, an upwardly extending metal bar 119. Each of these bars and its assembled parts are identical so that only one need be described. Each bar 119 is secured by means of screw bolts 121 passing through the bar and threaded in ribs 114 of mold member 82. At its upper end the bar 119 pivotally supports a lever 122 by means of screw bolt 123. Lever 122 carries a pivoted wedging member 124 by means of screw bolt 125. Wedging lever 124 has its lower inner end beveled at 126 and the lever 122 may have a fiber extension 127 for grasp by the hands of the operator.

The upper flange 107 of the fixed mold 82 also supports a pair of forwardly extending keeper frame members 128 spaced from it by a spacer 129. Keeper frame members 128 are joined by a keeper bar 130 which may be secured thereto by welding or any convenient fastening means. The operation of the securing means is as follows:

The wedging lever 124 engages the rib 114 of movable mold member 81. When the lever 122 is pulled downward by its handle 127, its outer side engages the bar 130 and its beveled surface 126 engages the mold. The proportions of the parts are such that wedging lever 124 is driven in between the mold 81 and bar 130 as a wedge to hold the mold members 81 and 82 together. The wedging action thus provided is sufficient to hold the two halves of the mold tightly together, but it is also adapted to take care of the expansion of the mold when the hot metal is poured into the mold.

The supporting framework for the ladle 10 also includes a pair of upwardly extending frame members 131, 132, secured by means of screw bolts to the ladle shell 39 at the bottom and to the band 51. The frame members 131, 132, preferably extend upward beyond the cover plate 70 where they may be bent outwardly slightly as indicated at 133, 134, and provided with the horizontal handle portions 135, 136.

Thus, the ladle and mold assembly has a handle 135, 136 at each end which may be grasped by a pair of operators or either of them in tilting the ladle and mold from the position of Fig. 3 to Fig. 5.

The mold 81 is also preferably provided with a pair of similar wedging members, one located at each side of the mold. In this case, the fixed mold is provided with a pair of forwardly extending strap members 137, 138, joined by a transverse strap 139 to form a keeper similar to 128, 129, 130, previously described.

A pivoted lever 140 comprising a pair of straps 141, 142 spaced and secured to a handlebar 143

is pivotally mounted on a frame member 144 by means of a screw bolt 145. A similar wedging member 146 extends between the straps 137, 138 and inside the strap 139 to engage the mold 81 and this wedging member 146 is pivotally mounted on lever 140 by screw bolt 147.

The frame member 144 may be a fixed member carried by the vertically extending bars 96. In this case the action of the wedging members is the same as described with respect to the wedging members 124 at the top, there being sufficient space between the handlebars 133, 134 and the mold to permit the necessary pivotal movement of the levers 140.

The interior of the mold cavity 106 in the mold member 81 likewise has its surface 148 in a substantially plane, smooth and polished condition, and the same is true of the inner surface 149 of the border flanges 116 at the end and both sides. Thus, the mold cavity 106 is of uniform cross-section from top to bottom and of uniform size.

The angular tilt of the mold cavity 106 with respect to the top of the ladle 10 is preferably such that when the ladle and mold are tilted, the free surface 150 of the molten metal 151 is adapted to well upward into the mold as the tilting progresses. The metal does not, therefore, run down to the end 149 of the mold cavity 106, but it moves upward into the cavity in a solid stream of uniform cross-section until the cavity is entirely filled and thereafter the continued tilting of the mold to the position of Fig. 5 permits a pressure to be placed on the metal in the mold which is determined by the head of metal above the mold cavity in the ladle in Fig. 5.

The cover plate 70 may be provided with a sliding cover 152 slidably mounted in guides 153 and provided with a slot 154 for engaging the gas burner pipe. The cover plate 152 may be provided with a handle 155 so that it may be slid to the open or the closed position by means of the handle. Thus, the burner opening may be closed, if desired, or, if necessary, to prevent the spilling of the metal out of the burner opening when the mold is tilted to the position of Fig. 5.

The method and operation of the apparatus is as follows: The ladle 10 is preferably preheated by means of the gas burner 54, the flame 53 of which plays into the cavity 43. Metal may be melted in one or more separate furnaces and a suitable supply of clean molten metal such as that provided by clean scrap or by ingots, may be placed in the cavity 43 after which the cover plug 48 and cover plate 70 may be secured in place. 55 The burner 54 is then again directed into the ladle cavity 43 and the flame is reflected from the free surface 150 of the molten metal into the mold cavity 106. This drives out the air and maintains a constant supply of neutral atmosphere, comprising exhaust gases. The pressure in the ladle is maintained slightly above atmospheric pressure so gas flows out crevices and air or oxygen cannot enter.

65 The apparatus may be preheated by means of this flame and by casting a few plates to bring it to the proper temperature. Thereafter, the casting operation may be carried out as follows: The mold having been closed and secured by means of the wedges, the ladle and mold are tilted gradually from the position of Fig. 3 in a counter-clockwise direction. As the ladle is tilted, the free surface of the molten metal 151 is, of course, maintained in horizontal position, and as the 70 mold is lowered, this free surface rises in the mold 75

cavity 106 due to the tilted position of the mold on the ladle.

The rising continues during the tilting operation until the mold is completely filled, without any splashing or separation of any part of the metal from the solid stream which enters the mold at the bottom and moves uniformly up through the mold until the mold is completely filled. The air or gas is expelled from the crack between the mold halves by the pressure of the molten metal which is sufficient to expel the air or gas.

As the tilting is continued downward to the position of Fig. 5, after the mold has been filled, a predetermined pressure is placed upon the metal in the mold and while the metal in the mold cools, pressure is continued until the shrinkage is completely taken up by the head of metal under pressure applied to the mold.

The casting in the mold freezes from the flat surfaces of the mold inward toward the center, and if the mold is tilted backward quickly enough, a hollow plate may be formed or a hollow tube may be formed by the metal which has congealed adjacent the walls of the mold, the molten metal running out of the inside to leave the casting hollow. Thus, the present invention may be used for making hollow castings or hollow tubes of any cross-section.

It should be understood that the cross-section of the mold may be circular for the making of hollow round pipes or it may be square or hexagonal or triangular or rectangular or any known or desired geometric form, the filling opening of the mold being of the same size and shape. The casting also congeals from the outer end of the mold, that is, the upper end in Fig. 3, toward the filling opening, the last to congeal being that portion adjacent the filling opening, so that additional metal is supplied to the casting as it congeals and all shrinkage is taken up.

In order to permit sufficient time for this congealing, the tilting action of the mold is so carried out that a predetermined number of seconds or counts are employed, or the mold may be held for a short time in the position of Fig. 5 before it is tilted back into the position of Fig. 3.

As soon as the mold is tilted back to the uppermost position the wedges are released and the movable mold member 81 is moved away from the fixed mold 82 and the movable mold is laid upon the horizontal supports 85. The casting will then be lying against the fixed mold member 82 and a very short sprue may extend into the discharge opening 55 of the ladle, but a minimum amount of sprue is present and there is a minimum amount of metal wasted by sprue action.

The result is a cast metal plate of homogeneous uniform grained structure without any segregations of impurities and without any pipe or cavity in the case of a solid casting. The present metal has been found to have an increased tensile strength and an increased purity over the metals cast according to the methods of the prior art, and the metals are particularly adapted to be used for drawing out metal cans or tubular containers such as the cans that are used for shields covering radio tubes of radio receivers.

The superlative product resulting from the use of this apparatus is attributed to the method of casting which may be carried out by the use of the present or other apparatus and which is summarized as follows:

The method is preferably carried out by means of a closed insulated ladle having a mold directly

attached to the discharge opening of the ladle so that there is practically no sprue attached to the casting. The mold is of metal of a higher melting point than the metal to be used in casting, such as cast steel, for casting aluminum, and the interior surface of the mold is smooth and polished on all sides.

The cross-section of the mold is preferably uniform from one end to the other for the casting of plates or other articles of uniform cross-section, and the filling opening of the mold, which is in registry with the discharge opening of the ladle, is of the same size as the cross-section of the mold. The discharge opening from the ladle is 15 preferably streamlined from the ladle cavity to the discharge opening of the ladle, which is of the same size as the filling opening of the mold.

It should be noted that the mold is preferably mounted in tilted relation to the ladle in such 20 manner that when the mold is tilted its filling opening is still the lowermost part of the mold and the free surface of the metal in the ladle may rise in the cavity of the mold uniformly until the mold is filled.

25 The ladle is filled to a predetermined level with clean molten metal, and the ladle is covered. Contact with the air is prevented by the gas flame, which plays on the free surface of the molten metal in the ladle and keeps the oxygen from that 30 surface to prevent or minimize oxidation. The ladle and mold are preheated either by suitable application of heat by flame or by providing a supply of super-hot metal to the ladle and making a few castings until the mold is suitably preheated. A pressure above atmospheric is maintained in the ladle to keep air out.

The casting operation is then carried out with the mold in direct connection with the ladle and by tilting the mold until the metal wells upward 40 into the mold in a solid unbroken stream without any agitation or churning. The congealation of the metal may begin as it enters the mold, but nevertheless the solid plug of congealing metal is driven upward into the mold by the pressure of 45 the metal in the ladle. The sliding engagement with the polished sides of the mold has a burnishing action on the finished casting.

50 The method of casting preferably includes the application to the mold of a gaseous flame, which is so adjusted that it produces a certain amount of soot in a very fine condition. This may be done by using an excess of gaseous fuel, such as illuminating gas, over the supply of oxygen. In 55 other words, the gaseous fuel predominates over the oxygen supply which would be required for perfect combustion, thereby producing a red flame.

55 This soot may uniformly coat the conduit leading from the ladle to the mold, and may coat the metal surfaces of the mold with a thin, fine layer of pure carbon. This carbon reduces the surface tension of the aluminum alloy filling the mold, and causes it to fill the mold more perfectly, but is sufficiently thin and fine so that it does not affect the surface of the casting, which conforms quite exactly to the cavity of the mold and provides a smooth and finished casting.

In addition to this, the carbon coating facilitates the separation of the mold from the casting, making the removal of the casting from the mold, or vice versa, easier than it would otherwise be.

Where the article to be cast is of uniform cross-section, so that congealation may start as the metal 75 enters the mold, the carbon coating acts as a

## 11

lubricant for the entering metal and aids in producing a more finished surface.

Before the casting operation is begun, the flame impinges on the free surface of the metal, and is reflected into the mold to preheat the mold, and especially to heat the filling aperture.

As the tilting progresses and the free surface covers the filling opening of the mold, the flame continues to heat the metal in the ladle, and when the mold and ladle have reached their extreme position the flame impinges against the wall of the ladle to continue the supply of heat for maintenance of the temperature of the molten metal in the ladle.

Thus the flame is automatically cut off from the filling aperture of the mold by the tilting action, and automatically re-applied to the metal when the ladle and mold return to their original position.

The temperature of the metal in the ladle is preferably maintained as close as possible to the melting temperature of the metal used in casting, that is, slightly above the solidifying temperature, so that when cast it solidifies quickly in the mold.

Less time is thus required for casting, and any tendency toward segregation is minimized by quicker congealation. The tendency toward segregation is greatest during congealation, and quicker congealation reduces or substantially eliminates segregation of impurities and segregation of ingredients of an alloy.

This "close to congealation" temperature is maintained by frequent measurement and constant observation of the indicated temperature of the molten metal in the ladle and of that in the furnace, by adjustment of the furnace and ladle temperature, by adjusting the heating arrangements of the ladle and of the furnace and by replenishing the ladle supply at proper time and temperature.

The ladle gas burner can be adjusted to higher or lower heat; or, if the metal in the ladle or furnace is too hot, a small solid piece of clean metal can be thrown into the molten metal to absorb heat by reason of its being heated and melted. The heat of fusion is taken from the surrounding molten metal, thereby reducing the temperature of all of the metal when molten.

For example, the silicon aluminum alloy 356 of the Aluminum Company of America has a composition of 7% silicon, 0.3% magnesium, and the rest aluminum. This alloy is stated to have a range of solidification of from 1130 degrees F. to 1075 degrees F. Using this alloy, the molten metal in the furnace may be maintained at a temperature not over 1300 degrees F. and not less than 1250 degrees F.

Under the same conditions, with small castings of irregular shape, the temperature of the metal in the ladle may be maintained at from 1175 degrees F. to 1200 degrees F.; but, if the machine is used for casting thin plates, the temperature of the molten metal in the ladle may be maintained at a temperature between 1225 degrees F. and 1250 degrees F.

Under these conditions the mold might be maintained, for example, at a temperature of from 600 degrees F. to 700 degrees F., preferably at about 650 degrees F.

It is also found that the proper temperatures for the molten metal in the ladle decrease during operation from the proper temperature which should be used in the beginning. For example, in the beginning, when the ladle is bringing the mold and other parts up to proper temperature, one

## 12

may start with a temperature of 1250 degrees F. with this alloy, and a half hour later reduce the operating temperature of the metal in the ladle to 1200 degrees F., and still later to 1175 degrees F. in the ladle, which may be then used for the substantially constant operating temperature.

The mold being attached directly to the ladle, with only one part detachable, keeps the mold hotter than it would otherwise be, but the mold is maintained at a temperature lower than that of the molten metal in the ladle, as indicated above, in order that it may cool the molten metal when the mold has been filled, and effect a quicker congealation.

In order that the mold may be cooler than the ladle parts, it is provided with some heat insulation between it and the ladle.

While in some embodiments of the invention artificial cooling by liquid or gas might be used, the temperature differential between the mold and the ladle and between the respective parts of the mold is preferably so regulated by the construction of the mold and ladle that no artificial cooling is needed for most castings.

In the apparatus illustrated the amount of metal used in the mold and the proportions of the mold and the amount of heat radiating surface provided are adapted to effect a proper cooling without necessity for artificial means, and these proportions are shown in the drawings.

The tilting is preferably carried out slowly so that the mold is filled slowly, and when the mold is filled the tilting is continued until the full pressure of the remaining metal in the ladle is placed on the metal in the mold.

Referring to Figs. 8 to 13, these figures show progressively the action of the flame and the molten metal during the casting operation.

In Fig. 8 the ladle is in upright position, and the flame is playing on the free surface of the metal, and is deflected into the mold.

Assuming that the dross on the surface has been skimmed off, the casting operation may then be commenced.

In Fig. 9 the tilting has progressed to such a point that the flame is cut off from the sprue by the fact that the free surface of the metal has begun to well up into the sprue or filling conduit.

As the tilting proceeds, it will be seen in Fig. 10 that the metal wells up into the mold. In this figure it has just begun to enter the mold. Further tilting causes the free surface of the metal to well up farther into the mold.

In Fig. 11 the mold is more than half way full.

In Fig. 12 the tilting has progressed to such a point that the mold is entirely full. This position is such that the free surface of the metal is above every part of the mold cavity.

The tilting is then continued to the position of Fig. 13, in which substantially every part of the mold cavity is below the main body of molten metal in the ladle. When a plate is being cast, as shown in Fig. 13, the mold cavity may be in substantially horizontal position.

In this position the pressure of the head of metal in the ladle is applied to the metal in the mold.

For some embodiments of the invention it is only necessary to proceed to the position of Fig. 13, but in others the tilting may be continued until the mold is substantially or entirely inverted, the mold being in vertical position, with the opening for the burner closed.

There are advantages in this additional step 75 of inverting the mold and casting after the filling

of the mold, as the natural heat gradient is then established from the lowermost and coldest part of the mold to the uppermost and hottest part of the mold near the ladle.

For example, at the temperatures mentioned, varying from 1250 degrees F., beginning, down to a stated temperature of 1175 degrees F., one hundred and twenty casting might be made per hour; and of course the major part of this time is spent in removing the casting from the mold and re-assembling the mold.

The exact amount of time which should be taken up in tilting the mold and the speed of tilting may be determined best by trial. For example, between five and ten seconds might be used in the timing of the down movement of the mold; but this may be varied by reason of the following conditions.

The thinner the cavity, the faster the filling and the freezing should be; and therefore the thinner castings must be made by tilting at a faster speed. The heavier the casting, the slower the filling may be, and in such case the mold may be brought down slowly, consuming as much as thirty seconds. The speed of the down movement is important; and if the downward movement is properly timed, the casting will be well formed.

In some cases, after the down movement has been completed, the mold may be lifted at once; but if the castings are heavier, the mold must be held down in the lower position for a certain number of seconds, until the congealing is accomplished inward from both sides of the mold, and back from the end of the mold to the filling aperture.

One advantage of holding the major axis of the mold in substantially horizontal position during congelation, or of merely moving it to the substantially horizontal position to fill the mold, is that all parts of the cavity will be subjected to substantially the same head of pressure by the metal in the ladle, because they are at the same level, and the pressure should be the same in a plane parallel to the free surface and at a predetermined distance below the free surface.

The tilting is preferably carried out slowly so that the mold is filled slowly and when the mold is filled, the tilting is continued until the full pressure of the remaining metal in the ladle is placed on the metal in the mold.

The metal in the mold then congeals from the large plane flat surfaces of the mold inward toward the center and from that end of the mold remote from the filling opening back to the filling opening. As the cooling of the casting takes place and the congelation takes place, further metal is supplied to the casting to take up all shrinkage, also without any splashing or other disturbing action, and the ladle and mold are preferably held with the mold in downward position and full metal pressure applied for a short time until congelation takes place. The timing depends upon the metals which are being cast and upon the characteristics and thickness of the mold and the temperatures employed.

When hollow castings, such as tubes or hollow plates, are to be made, the ladle and mold are tilted backward to the uppermost position immediately without any delay and the thickness depends upon the temperatures and the speed of tilting and re-tilting. This may quickly be determined by trial, and it is not possible to specify any given time except with a given apparatus at a given temperature.

There is no spouting of the metal out of a nozzle into the mold, no forming of drops or separate oxidized particles, and the only part of the casting which is subjected to air is that small area at the end of the solid advancing stream of metal in the mold and that end portion becomes the end of the casting.

The present method may be used for casting various types of metals and alloys, and it is only necessary to use suitable molds of metal of a melting point higher than the metal to be used in casting.

As soon as the assembly is tilted back to the upper position, the wedges are released and the movable mold members withdrawn and the casting is pried loose from its position against the fixed mold member with its end sticking into the discharge opening of the ladle. It may then be laid upon a flat surface to cool gradually and to shrink without producing strains that might otherwise occur if it were left in the mold. The castings may be placed in a suitably heated furnace to cool gradually, and are preferably protected, in any event, from drafts and irregular cooling influences.

When the metal is to be used for drawing metal containers, the plates may be taken to a punching machine, and metal slugs may be punched out of the casting. The metal slugs are then placed in suitable dies, and the drawn cans or containers may be drawn without any preheating. The metal is easily worked, and it may be drawn cold into containers or members of various different sizes and shapes.

As distinguished from tubular members made out of blanks that came from commercial metal, this drawing may be accomplished without big strain on the machinery on account of the fact that the metal is more easily worked. The large percentage of defective boxes or containers which resulted from the methods of the prior art is not present according to my method, as practically all of the containers are perfect. There is a large saving in the cost because clean scrap or ingot metal is much cheaper than the sheet metal of which the blanks were made according to the prior art.

It will thus be observed that I have invented an improved method of making castings and making drawn metal containers by means of which more perfect and more economical containers may be made, with less metal and at a lower cost. There is a minimum amount of waste by reason of the fact that there is a minimum amount of sprue, and the metal has a uniform-grained homogeneous structure without any segregated impurities or cavities or other defects.

As the mold opening is of the same size as the ladle discharge opening, the metal may well up into the mold without any agitation or spouting or splashing, and there are no small particles or drops formed which may harden first and be oxidized on their outside and then incorporated in the casting. The casting comprises one uniform stream of metal which slides into the mold and is burnished to a smooth polished finish.

The present plates may be rolled by the usual rolling machinery into sheets of any desired gauge and width, but the amount of rolling that is necessary is very small because of the initial thin character of the plate castings. A large amount of rolling is eliminated, and the cost of the metal sheets is greatly reduced.

According to my method, no part of the melted

metal is ever separated from the compact stream of melted metal welling up into the mold. If any part of the metal becomes separated from the stream, it would be surrounded with oxygen and become oxidized, and would not fuse again in the mold to make such a homogeneous structure as I am able to secure.

While I have illustrated a preferred embodiment of my invention, many modifications may be made without departing from the spirit of the invention, and I do not wish to be limited to the precise details of construction set forth, but desire to avail myself of all changes within the scope of the appended claims.

Having thus described my invention, what I claim as new and desire to secure by Letters Patent of the United States is:

1. A permanent mold assembly comprising a metal plate having a mold filling opening therein, a pair of longitudinally extending metal frame members carried by said plate, and a pair of transversely extending frame members projecting transversely from said plate and secured to said longitudinal frame members, a mold member comprising two halves, one of said halves fitting between said longitudinally extending frame members adjacent said filling opening and having its inner surface in registry with the edge of said filling opening, said transversely extending frame members having a cross head adapted to support said one half of the mold, the second half of said mold member being provided with a cavity and also fitting between said longitudinal and transverse frame members against the first half of the mold, said cavity being formed with an opening at its lower end in registry with said filling opening in said plate, and means for securing said mold halves together, said latter means comprising a pivoted lever carried by the first mold half, and a cross bar carried by said first mold half, a wedging member pivoted on said lever, and adapted to be engaged between the cross bar and the second mold half.

2. A permanent mold assembly comprising a metal plate having a mold filling opening therein, a pair of longitudinally extending metal frame members carried by said plate, and a pair of transversely extending frame members projecting transversely from said plate and secured to said longitudinal frame members, a mold member comprising two halves, one of said halves fitting between said longitudinally extending frame members adjacent said filling opening and having its inner surface in registry with the edge of said filling opening, said transversely extending frame members having a cross head adapted to support said one half of the mold, the second half of said mold member being provided with a cavity and also fitting between said longitudinal and transverse frame members against the first half of the mold, said cavity being formed with an opening at its lower end in registry with said filling opening in said plate, and means for securing said mold halves together, said plate also having a transverse shoulder member secured on the plate to engage the outer surface of the second half of the mold to hold the parts of the mold together at said plate.

3. A permanent mold assembly comprising a

metal plate having a mold filling opening therein, a pair of longitudinally extending metal frame members carried by said plate, and a pair of transversely extending frame members projecting transversely from said plate and secured to said longitudinal frame members, a mold member comprising two halves, one of said halves fitting between said longitudinally extending frame members adjacent said filling opening and having its inner surface in registry with the edge of said filling opening, said transversely extending frame members having a cross head adapted to support said one half of the mold, the second half of said mold member being provided with a cavity and also fitting between said longitudinal and transverse frame members against the first half of the mold, said cavity being formed with an opening at its lower end in registry with said filling opening in said plate, and means for securing said mold halves together, said plate also having longitudinally extending frame members provided with a cross-bar and of sufficient length to support the second half of the mold when it has been separated from the first half.

4. A permanent mold assembly comprising a metal plate having a mold filling opening therein, a pair of longitudinally extending metal frame members carried by said plate, and a pair of transversely extending frame members projecting transversely from said plate and secured to said longitudinal frame members, a mold member comprising two halves, one of said halves fitting between said longitudinally extending frame members adjacent said filling opening and having its inner surface in registry with the edge of said filling opening, said transversely extending frame members having a cross head adapted to support said one half of the mold, the second half of said mold member being provided with a cavity and also fitting between said longitudinal and transverse frame members against the first half of the mold, said cavity being formed with an opening at its lower end in registry with said filling opening in said plate, and means for securing said mold halves together, said mold member being constructed of steel plates formed with transversely and longitudinally extending spaced reinforcing ribs.

CARL WESSEL.

#### REFERENCES CITED

The following references are of record in the file of this patent:

#### UNITED STATES PATENTS

| Number    | Name     | Date          |
|-----------|----------|---------------|
| 2,333,286 | Wessel   | Nov. 2, 1943  |
| 440,801   | Adams    | Nov. 18, 1890 |
| 954,368   | Allison  | Apr. 5, 1910  |
| 1,533,734 | Gotze    | Apr. 14, 1925 |
| 2,106,614 | Lindner  | Jan. 25, 1938 |
| 94,170    | Pedder   | Aug. 31, 1869 |
| 1,138,443 | Bierbaum | May 4, 1915   |
| 1,368,445 | Little   | Feb. 15, 1921 |
| 48,215    | Sexton   | June 13, 1865 |
| 905,287   | Chipman  | Dec. 1, 1908  |
| 2,134,829 | McWane   | Nov. 1, 1938  |
| 2,223,617 | Johnston | Dec. 3, 1940  |
| 2,209,519 | Halbrow  | July 30, 1940 |